

Dec. 31, 1929.

A. ELMENDORF

1,741,760

INSULATING BUILDING MATERIAL AND METHOD OF MAKING THE SAME

Original Filed May 31, 1927



Inventor:  
Armin Elmendorf,  
by Wm. F. Freudenberg, atty

## UNITED STATES PATENT OFFICE

ARMIN ELMENDORF, OF CHICAGO, ILLINOIS

## INSULATING BUILDING MATERIAL AND METHOD OF MAKING THE SAME

Application filed May 31, 1927, Serial No. 195,265. Renewed May 31, 1929.

The present invention has for its object to produce a novel building material that may be produced at comparatively low cost, be very effective as an insulation against 5 heat and cold, which may be sawed in the same way as lumber, which will be weather-proof so that it will not be injured by exposure to the weather pending the placing of the same in a wall or other structure, which 10 will not expand or contract upon changes in its moisture content or in the moisture in the surrounding atmosphere.

A further object of the present invention is to produce a novel and comparatively inexpensive block possessing heat insulating properties to a high degree, and having the qualities or characteristics required for an efficient roof foundation.

The various features of novelty whereby 20 my invention is characterized will herein-after be pointed out with particularity in the claims; but, for a full understanding of my invention and of its objects and advantages, reference may be had to the following detailed description taken in connection with the accompanying drawing, wherein:

Figure 1 is a perspective view of a finished block made in accordance with my invention; Fig. 2 is a perspective view of the block, on 30 an enlarged scale, portions being broken away to illustrate the manner of building up the block; Fig. 3 is a transverse section through a modified form of block; and Fig. 4 is a transverse section through a still further 35 modified form of block, only a fragment of the block being shown.

In carrying out my invention, I make use of fibrous vegetable matter, preferably stems 40 consisting of an outer skin or shell filled with pith. I believe corn stalks will be used most largely for the manufacture of my improved blocks. Therefore, since my invention can be fully explained in connection with the manufacture of blocks from corn stalks, for 45 the sake of brevity I refer to the base or body material as corn stalks, although other fibrous vegetable material having the required properties may be employed.

In the manufacture of the blocks, the corn 50 stalks, placed side by side, are pressed into a

compact mass which is then sawed into sections or planes at right angles to the length of the stalks. A binder or bonding material, preferably of gypsum or magnesite, is applied to the sawed faces, the binder being 55 then covered with paper or the like, preferably waterproofed paper. The paper is preferably applied while the binder is still plastic. Upon the setting of the binder, the pieces of corn stalk will be held under compression. At this stage of the operation the blocks or slabs may be of finished size or shape or they may be of approximately the finished width but longer than an individual block is to be, depending on the process of 60 manufacture. If the process of manufacture be such that slabs longer than a single block are produced, the slabs are sawed into the desired lengths, producing two sawed edges, and then the other two edges may be trimmed 65 if desired, to make them flat. After the edges have been trimmed they present faces that to the eye appear to be composed entirely of pith, since the trimming cuts are made lengthwise of the stalks and thus divide the 70 skins or shells of the stalks lengthwise. The edges whether trimmed or not, are then covered and the individual blocks are ready for use.

Referring to Figures 1 and 2 of the drawing, A represents a finished block or slab. The core 1 of the block or slab comprises the stalks or stems arranged side by side, approximately parallel with each other, and compressed into a compact mass, as shown in 80 Fig. 2. 2 and 3 represent the top and bottom layers of binding material, in this case of cement; while 4 and 5 are the paper coverings. The edges of the block are coated with cement, as indicated at 6, and the cement is in 85 turn covered with the waterproof paper 7 or other suitable material.

The blocks may be made of the same thickness as the depth of the studding employed in the construction of buildings, so that they 90 may be fitted in between consecutive studding elements and form with the latter a solid wall of uniform thickness; or the blocks may be made thinner if desired. The blocks may be sawed to fit spaces that are to receive them. 100

Each block is therefore made waterproof, and it will not become damaged or distorted when exposed to the weather as such material must be in preparing for and constructing buildings.

5 It will be seen that the size and shape of each block are permanently fixed. There is no appreciable shrinkage of the fibres in the direction of their length, and any transverse shrinkage which might otherwise take place 10 is prevented by the layers of cement fixed thereto. Therefore, after my improved blocks have been built into a structure, there is no danger that openings will be produced 15 between the studding and adjacent blocks, due to shrinkage of a block.

Another valuable characteristic of my improved block is its ability to localize moisture that may perhaps enter the same through a 20 damaged sheathing. The skins or shells of the stalks are waterproof, so that if water leaks into the core it will be confined within those tubular skins into which it originally enters, and cannot spread. Furthermore if 25 an entire block should be wet, the sheathings on adjacent blocks will protect the latter against the entry into the same of moisture from the wet block.

30 My improved blocks may be used for making roofs, taking the place of wooden sheathing; the blocks, preferably in the form of slabs, being simply placed on wooden beams spaced at the proper distances apart.

In order to give the blocks greater mechanical strength, that will permit them to 35 carry a load when used in roofs, the bottom layer 8 of cement, as best shown in Fig. 3, may contain metal reinforcing, conveniently in the form of wire mesh 9. The top and bottom faces of the roof slabs or blocks may be 40 covered with waterproof paper 4 and 5. Instead of employing paper that has been saturated with asphalt or other waterproofing material, two-ply paper with a layer of asphalt or waterproofing material between the 45 same may be employed.

The edges of blocks or slabs of this type may first be coated with asphalt, as indicated at 10, emulsified asphalt being preferably employed. A layer 11 of cement is then 50 applied over the asphalt; the cement being preferably gypsum or magnesite in the form of a wet paste. In fact, I prefer to use a gypsum paste containing wood fibre.

55 These roof slabs may be laid side by side, with the reinforced faces down, and a protective covering placed over the same. Such covering may consist of a thin layer of asphalt overlaid with any desired number of 60 sheets of roofing felt.

Each corn stalk section in a block or slab constitutes a column possessing considerable compressive strength. Therefore, when the 65 blocks or slabs are used as roof foundations,

they are sufficiently strong to carry the usual roof loads and traffic.

Instead of cement as a binder, I may use a hard asphalt as shown in Fig. 4. Referring to Fig. 4, the core 1 is coated on the top and 70 bottom faces with asphalt as indicated at 12, the asphalt being covered with paper 13. The edges of the block may be coated with asphalt 14, dusted with talc or the like.

75 While I have illustrated and described with particularity only a single preferred form of block, with a few slight modifications, I do not desire to be limited to the specific details thus illustrated and described; but intend to cover all forms and processes coming within 80 the definitions of my invention constituting the appended claims.

I claim:

1. The method of making a building block, comprising the compacting of a mass of 85 fibrous material in which the fibres are parallel, cutting the mass into slabs along planes transverse to the fibres, and applying a binder to the faces thus formed.

2. The method of making a building block 90 of corn stalks, comprising the compacting of a mass of corn stalks arranged parallel with each other, severing the mass into slabs along planes transverse to the length of the stalks, and covering the faces thus formed with a 95 binder.

3. The method of making a building block, which consists in compacting a mass of 100 fibrous material in which the fibres are parallel, cutting the mass into slabs along planes transverse to the fibres, applying a binder to the faces thus formed, cutting the slabs into blocks, and covering the blocks with a water 105 proof sheathing.

4. The method of making a building block, 105 which consists in compacting a mass of parallel vegetable stems, cutting the mass into slabs along planes at right angles to such stems, applying cement to the faces thus formed, dividing the slabs into blocks of the 110 desired size, and sheathing the blocks with a waterproof material.

5. The method of making a building block, which consists in compacting a mass of 115 fibrous material in which the fibres are parallel with each other, cutting the mass along planes transverse to the fibres into slabs, applying cement to the faces thus formed, covering the cement with a waterproof material, and cutting the slab into blocks and trimming 120 the edges of the blocks.

6. The method of making a building block, which consists in the compacting of a mass of fibrous material arranged parallel with each other, forming blocks by cutting the 125 mass into sections having faces lying in planes transverse to the fibres, and encasing said blocks in a waterproof sheathing.

7. The method of making a building block, 130 which comprises the compacting of a mass of

fibrous material arranged parallel with each other, forming blocks by cutting the mass into sections having faces lying in planes transverse to the fibres, and bonding the ends of 5 the fibres lying in said faces.

8. The method of making a building block, which consists in compacting a mass of fibrous material in which the fibres are parallel with each other, cutting the mass along 10 planes transverse to the fibres into slabs, applying cement to the faces thus formed, covering the cement with a waterproof material, cutting the slab into blocks and trimming the edges of the blocks, and sheathing the edges 15 of the blocks with a waterproof material.

9. A building block comprising a compacted fibrous mass having the fibres arranged parallel with each other, bonding means for the fibres covering the faces containing the 20 ends of the fibres, and a paper covering over the whole.

10. A building block comprising a compacted fibrous mass having the fibres arranged parallel with each other and cut off 25 at the ends to form flat faces on the block, and a cement covering for the faces containing the ends of the fibres.

11. A building block comprising a compacted fibrous mass having the fibres arranged parallel with each other and cut off 30 at the ends to form flat faces on the block, bonding coverings for the faces containing the ends of the fibres, and reinforcing tension members embedded in one of said coverings.

35 12. A building flat relatively thin block comprising a compacted mass of fibres arranged at right angles to the two opposed flat faces of the block and a thin binding layer of cement covering said faces.

40 13. A building block comprising a core composed of a compacted mass of corn stalk lengths arranged at right angles to and terminating in two opposed faces of the block, binding coverings for said faces, and reinforcing tension members embedded in one of 45 said coverings.

14. The method of making a building block, comprising the compacting of a mass of fibrous material in which the fibres are 50 parallel, cutting across the fibres to produce a block having opposed flat faces containing the ends of the fibres, and applying a binder to said faces.

In testimony whereof, I sign this specification.

ARMIN ELMENDORF.